

R. H. STEVENS.

## PROCESS FOR AMALGAMATING METALS.

APPLICATION FILED AUG. 29, 1918.

1,384,683.

Patented July 12, 1921.

Fig. 1.



Fig. 2.



Inventor

Ransom H. Stevens

By James T. Pickleman  
His Atty

# UNITED STATES PATENT OFFICE.

RANSOM H. STEVENS, OF LOS ANGELES, CALIFORNIA, ASSIGNOR OF ONE-THIRD TO  
W. R. CROWELL AND ONE-THIRD TO L. C. COMER, BOTH OF LOS ANGELES, CALI-  
FORNIA.

## PROCESS FOR AMALGAMATING METALS.

1,384,683.

Specification of Letters Patent. Patented July 12, 1921.

Application filed August 29, 1918. Serial No. 251,909.

To all whom it may concern:

Be it known that I, RANSOM H. STEVENS, a citizen of the United States, residing at Los Angeles, in the county of Los Angeles, 5 State of California, have invented new and useful Improvements in Processes for Amalgamating Metals, of which the following is a specification.

This invention relates to processes for 10 amalgamating metals; and although the process is generally intended and adapted to all kinds of amalgamation work—that is the gathering of metallic particles into the body of a liquid metal mass—coalescing the 15 metallic particles with that mass—the process is particularly designed for the efficient recovery of gold that has been "floured" with mercury and is recoverable only with difficulty by other methods.

20 The process has fundamentally to do with the passing of a current or stream of pulp liquid through an amalgamating metal or metals (such as mercury, etc.,) under the action of an electric current, in such a way 25 that the stream of pulp liquid and suspended amalgamable metals passes through an electric current immediately before or at the time of entering the amalgamating metal. The process may be effectively carried on 30 in an apparatus wherein the pulp liquid stream passes under the lower edge of a wall which dips into the metal bath, such as a mercury bath. Electrodes are provided to apply an appropriate current to the flowing 35 pulp liquid; and the amount of current is regulated in accordance with the character and amount of metal to be recovered, the speed of the pulp liquid stream, and generally in accordance with the size and 40 capacity of the apparatus. The process will be best understood when it is explained in connection with a suitable form of apparatus; such apparatus being illustrated in the accompanying drawings where Figure 1 is 45 a vertical section and perspective of the apparatus; and Fig. 2 is an enlarged diagram illustrating the action.

In the drawings I show a box having a back wall 10, side walls 11 and a front over- 50 flow wall 12. A partition wall 13 forms with the back and side walls a chamber in which pulp liquid 14 is maintained at any suitable level L. The fluid stands at level L<sup>1</sup> in the chamber in front of partition wall

13, level L<sup>1</sup> being determined by the height 55 of over-flow wall 12. The height of level L above level L<sup>1</sup> is governed in accordance with the amount of flow desired under the lower edge 13<sup>a</sup> of partition wall 13. With any given apparatus the rate of flow de- 60 pends entirely upon the height of level L.

Lower edge 13<sup>a</sup> of partition wall 13 dips into a mercury or other amalgamating metal bath shown at 15, contained in a metal pan 16 having an electric connection means at 17. 65 This metal bath may extend its metallic surface somewhat to each side of the wall 13<sup>a</sup>, so that a considerable metallic surface may be exposed and so that a considerable mass of metal may be placed in the amalgamating 70 bath without having an excessive distance between the lower edge 13<sup>a</sup> and the bottom of pan 16. It is an object to have this distance comparatively small so that the stream of pulp liquid is spread out into thin 75 stream in passing under the wall 13; so that all parts of the metal carrying pulp liquid are intimately exposed to the amalgamating action of the metal in the bath. The efficient dimension for this height of opening having 80 been determined, the capacity of the apparatus may be increased by increasing the length of the passage space under wall edge 13<sup>a</sup>; that is, by increasing the dimension of 85 the apparatus in a direction at right angles to the surface of the drawing. Thus in practice the opening below the edge 13<sup>a</sup> may become a long, narrow opening.

On the opposite sides of partition wall 13, above its lower edge, are two electrode plates 90 20, which may preferably be of carbon or any other suitable conducting material. Connections 21 extend from these electrode plates to an electrical connection at 22. The electrode plates extend the whole length of 95 partition wall 13 and the lower edges of the electrode plates are at a suitable distance above the level of the liquid bath 15. Positive electrical connection is made at 22 and negative electrical connection is made at 17; so that 100 current flows downwardly from the two electrode plates 20 to the surface of metal 15, through the pulp liquid; and the metal carried in suspension in the fluid will thus be subjected to the electrical action just as it 105 enters and just as it leaves the amalgamating liquid. The metal is amalgamated into the amalgamating liquid and remains in the

bath 15, while the spent pulp liquid passes into the front chamber and overflows the wall 12.

In operating this apparatus, and carrying on my process, I first prepare the ore by forming a thin pulp liquid with water; and this fluid, with its suspended ore and metallic particles is delivered into the rear compartment of the device in such quantity as to maintain a uniform level. The electric current is turned on and the pulp liquid flows through the zone of electric current and through the amalgamating metal, being spread out into a thin stream while it passes through the space between the wall 13 and the amalgamating metal. It will be noted that the pulp liquid is spread out into a comparatively thin stream also where it passes the electrodes; the distance between the electrodes and the amalgamating metal being gaged to obtain maximum electrical effect on the pulp liquid as it passes through the space denoted 25. The current flow is most concentrated directly down onto the mercury; but it may also flow somewhat diagonally outwardly to the outer parts of the mercury bath and also to the exposed edge portions of the pan 16. The head of liquid in the rear column at 14 causes the mercury surface to be displaced downwardly on the rear side of the wall 13; so that the pulp liquid may flow under the wall. This displacement, when the pulp liquid stream is flowing, may be more or less exclusively near and under the wall 13; so that the situation will be more or less like that illustrated in Fig. 2. However, in the displacement space near and under the wall 13, the pulp liquid is at all times in intimate contact with the amalgamating liquid. Consequently, it will be seen, the pulp is subjected to electrical action simultaneously with its subjection to intimate relation to the mercury. The electrical current not only flows through the stream to the body of mercury beneath but flows through a stream of pulp liquid that is more or less intermingled with and in intimate contact with the mercury. Substantially all of the metal is caught and held in the amalgamating bath. This is particularly true, and the process is particularly efficacious, as applied to ores containing gold that has been floured with mercury. Under the action of the electrical current and the amalgamating action of the mercury bath, the floured gold is readily amalgamated and coalesced into the body of mercury, leaving the spent ore in suspended form to overflow wall 12. Under different conditions the amount of voltage and amperage of the electric current will be different; depending upon the amount and character of ore and the speed at which it is put through the apparatus. In a typical small sized apparatus where the passage under the

lower edge 13<sup>a</sup> of the partition wall is from one-half to three-quarters of an inch in height, where the wall 13 dips one-eighth to one-quarter of an inch into the mercury, and where the electrodes are one-quarter to one-half an inch above the mercury, using mercury in the bath 15 and operating upon floured gold ore, a voltage of from ten to twenty volts may be sufficient; the amperage will depend upon the conductivity of the fluid, but in a typical case may be approximately one to two amperes for each foot in length of the partition wall.

Actual tests of the method and apparatus hereinbefore described have clearly demonstrated the practicability and effectiveness of the invention.

The effect of passing the electric current through the pulp liquid prior to the latter coming into contact with the mercury seems to carry the metal particles toward the mercury and this action is found to be more effective in that portion of the flow of pulp liquid which is toward the mercury than in the portion flowing away therefrom. That is, such effect is greater at the left hand side of the partition in Fig. 1 than at the right thereof. The combined physical movement of the pulp liquid toward the mercury and the movement of the electric current through the pulp liquid toward the mercury causes the metal particles to be carried into direct and intimate contact with the mercury.

Having described my invention, I claim:

1. The process of amalgamating metals which embodies passing a liquid containing the metal to be amalgamated beneath a partition that extends below the level of a body of an amalgamating substance, the upper surface of the amalgamating substance being depressed beneath the partition by the weight of the body of liquid to form a passage through which the liquid flows in contact with the amalgamating material; and causing an electric current to flow through the liquid prior to and while it is in condition with the amalgamating substance.

2. The process of amalgamating metals which embodies passing a liquid containing the metal to be amalgamated beneath a partition that extends below the level of a body of an amalgamating substance supported by a receptacle constituting a portion of an electric circuit, the upper surface of the amalgamating substance being depressed beneath the partition by the weight of the body of liquid to form a passage through which the liquid flows in contact with the amalgamating material, and causing an electric current to pass through the liquid to said receptacle both above the level of the amalgamating substance therein and through said substance.

3. The process of amalgamating metals which embodies passing a liquid containing the metal to be amalgamated beneath a par-

tion that extends below the level of a body of an amalgamating substance supported by a receptacle constituting a portion of an electric circuit, the upper surface of the amalgamating substance being depressed beneath the partition by the weight of the body of liquid to form a passage through which the liquid flows in contact with the amalgamating material, and causing an electric current to pass from opposite sides of the parti-

tion to said receptacle through the amalgamating substance and superposed stream of liquid.

In witness that I claim the foregoing I have hereunto subscribed my name this 24<sup>15</sup> day of August, 1918.

RANSOM H. STEVENS.

Witness:

VIRGINIA I. BERINGER.